

Patented July 10, 1928.

1,676,929

UNITED STATES PATENT OFFICE.

BY RAMJI D. SAKLATWALLA, OF CRAFTON, PENNSYLVANIA.

COPPER CHROMIUM FERROUS ALLOYS.

No Drawing.

Application filed April 7, 1924. Serial No. 704,633.

This application is a continuation in part of my copending application Serial No. 584,552, filed August 26, 1922. The claims in said prior application are directed to the proportions of copper and chromium without reference to the silicon, whereas the claims of the present application are directed particularly to the inclusion of the silicon in a copper-containing copper-chrome ferrous alloy.

The present invention relates to copper chromium ferrous alloys, and particularly to alloys containing a sufficient percentage of chromium and copper as to render them substantially non-corrodible and acid resistant.

The invention relates more especially to alloys containing over 2 or 3% chromium, and particularly to so-called stainless steels which usually contain from 8 to 25% of chromium. I have found that if the proper amount of copper be added to such chrome steels, the stainless qualities are not only enhanced, but the steel is made substantially resistant to acids. The copper also tends to make the steel more malleable and easier to work. I have also found that the malleability and resistance to corrosion may be increased, particularly with high carbon steels, by the presence of silicon with the copper.

The so-called stainless steels usually contain between 8 and 25% of chromium together with hardening carbon usually .1% or over. These steels are stainless or rustless only when hardened and polished, and they are not resistant to strong acids. I have found that by the addition of from .15 to 5% of copper, such steels are made more rust and stain resisting and also acid resistant. The acid resistant properties begin to appear with the addition of about 1.5% of copper, but are not so markedly present until about .5% of copper is added. I prefer to use about 2 to 3% of copper. Such percentage of copper renders the steels resistant to stain and rust, not only when hardened and polished, but also when in the annealed and roughened state. The steels are also extraordinarily resistant to strong acids, such as hydrochloric and sulphuric. They are resistant to corrosion in those industrial atmospheres where the air is contaminated with sulphurous and combustion gases. The copper also increases the flame resisting properties of such steels by increasing their

resistance to oxidation at high temperature. While the stain, rust and acid resisting qualities of my copper chromium steel are especially pronounced in the so-called stainless steel range of chromium, namely 8% or over, they show extraordinarily good resistance to corrosion and acid attack when containing lower percentages of chromium, say down to 2 or 3%, although it is not so strongly resistant as with the higher percentages of chromium.

The copper, in addition to rendering the alloy more resistant to corrosion and acids, increases its malleability, ductility and dynamic strength.

The susceptibility to corrosion and acid attack increases with the amount of carbon content so that to obtain the same corrosion and acid resisting qualities, the amount of chromium and copper should be increased for the higher carbon contents. The higher carbon content, of course, also tends to make the alloy harder and more difficult to fabricate. The effect of the higher carbons may be counteracted to a considerable extent by the addition of silicon to the alloy in percentages varying from .5 to 6%, preferably about 1 to 3%. The silicon apparently counteracts the effect of the carbon and tends to make the alloy non-corrosive and more malleable so that it may be more readily rolled and fabricated.

In forming the alloy, sufficient carbon should be present to give the desired tensile strength and hardness desired. The carbon will in general range from .1 up as high as in the neighborhood of 2% for special steels. The chromium and copper apparently react with the carbon and tend to maintain it as hardening carbon and prevent its segregation as cementite or graphite. This permits the alloy to be quenched more slowly than plain carbon steel. The copper and chromium hold the carbon in its combined hardening form at relatively high temperatures, which is of considerable advantage in tool and roll steels which are subjected to heat, because the steel will not soften in use at a temperature which would soften plain carbon steel. This ability of the copper and chromium to hold the carbon in its combined state is particularly valuable in high carbon steels or high carbon cast iron, in that a high percentage of carbon may be kept in the hardening state so as to form a very hard article.

While the present invention has been described with particular reference to its application to the so-called stainless or rustless steels, it may be applied to other steels and irons.

The presence of the copper in the proportions specified does not materially interfere with any properties imparted to the steel by reason of its carbon and chromium contents. On the contrary, the copper content acts in an additive manner toward augmenting the tensile strength derived from the carbon and chromium contents, and also increases the ratio of elastic limit to tensile strength. Also, the presence of copper does not interfere in any way with the possibilities of heat treatment, thus allowing a latitude in the direction of a variation of physical properties.

The proportions of the chromium, copper, carbon and silicon may be varied over fairly wide ranges within the limits described, so that steels of different physical properties may be produced, which will, however, have the desirable stain, rust and acid resisting properties.

In the foregoing description no reference has been made to the presence of other elements, such as manganese, sulphur, phosphorus, etc., which are always present in steels and cast irons, as their presence to the usual extent does not interfere with the physical or non-corrosive properties of the alloys.

The present invention is not limited to the exact proportions above set forth as its preferred embodiment, but may be otherwise embodied within the scope of the following claims.

I claim:

1. A ferrous alloy containing carbon,

about 8 to 25% chromium, .5 to 5% copper and 1 to 3% silicon.

2. A resistant-surface alloy of iron comprising, in combination with the iron, silicon from .50% to 6%, chromium from 3% to 30% and copper from 10% to 2%.

3. A ferrous alloy containing from .1% to 2% carbon, from 2% to 25% chromium, from .15% to 5% copper and from .5% to 6% silicon.

4. A ferrous alloy containing from 2% to 25% chromium, from .15% to .5% copper and from .5% to 6% silicon, together with carbon.

5. A ferrous alloy containing over 2% chromium but not over the percentage of chromium in stainless steels, from .15% to 5% copper and from .5% to 6% silicon, together with carbon.

6. A ferrous alloy consisting principally of iron and containing over 2% chromium, .15% to 5% copper and .5% to 6% silicon, together with carbon.

7. A resistance surface alloy of iron comprising in combination with the iron, silicon from 1% to 6%, chromium from 2% to 10%, copper from .5% to 5%.

8. As a new product, an alloy steel comprising silicon from 1% to 6%, chromium from 2% to 10%, copper from .5% to 5%, carbon from .05% to 1%, and the balance iron.

9. As a new product, an alloy steel comprising silicon from 1% to 6%, chromium from 2% to 10%, copper from .5% to 5%, carbon from .1% to 1%, and the balance iron.

In testimony whereof I have hereunto set my hand.

BYRAMJI D. SAKLATWALLA.